

## 1

2,864,766

**UTILIZATION OF MIXTURES OF ORGANIC AND INORGANIC ACIDS IN THE PREPARATION OF GREASES****Arnold J. Morway, Clark, N. J., assignor to Esso Research and Engineering Company, a corporation of Delaware****No Drawing. Application November 30, 1955  
Serial No. 550,176****9 Claims. (Cl. 252—36)**

This invention relates to lubricating grease compositions, and more particularly to lubricating oil thickened to grease consistency with neutralized blends or mixtures of low molecular weight carboxylic acids and mineral acids and stabilized with a minor amount of an aluminum soap of a high molecular weight carboxylic acid.

In brief, this invention pertains to the stabilization of lubricating grease compositions containing as the thickening agent an alkaline earth metal neutralized blend of a low molecular weight carboxylic acid, e. g. acetic acid, with a strong inorganic acid, e. g. phosphoric acid, and an aluminum soap of a high molecular weight fatty acid, e. g. aluminum stearate.

When the metal salts of low molecular weight carboxylic acids are dispersed in lubricating oils, the resulting composition tends to be rather unstable when employed under ordinary lubricating conditions. A composition of this type loses its solid structure and settles out large clumps of the metal salt when the lubricant is employed at temperatures where dehydration will occur.

The use of small amounts of metal salt of phosphoric acid in lubricating grease compositions containing large amounts of metal soaps as the thickening agent has previously been suggested in the art. In U. S. Patent No. 2,513,680 to Schott and Armstrong, for example, less than about 2.0% by weight of calcium phosphate is employed to improve the "skin hardening" and storage stability properties of calcium base greases.

It has now been found that a large amount of a mineral acid in combination with a low molecular weight carboxylic acid can effectively thicken a lubricating oil to grease consistency provided that a minor amount of aluminum soap of a high molecular weight acid is employed in conjunction therewith. The aluminum soap appears to prevent the grease composition from separating oil during storage over long periods of time and to prevent the thickening agent from agglomerating and settling out of the lubricating composition.

It is not known what reactions the strong inorganic acid enters into during the grease preparation method of this invention. When nitric acid is employed, for example, the resulting grease composition had a distinctive red color, as hereinafter shown. However, for the purposes of this invention it is sufficient to note that lubricating compositions encompassed therein are prepared by utilizing blends or mixtures of the low molecular weight carboxylic acids and mineral acids.

Suitable low molecular weight carboxylic acids include saturated and unsaturated aliphatic carboxylic acids having from about 1 to about 3 carbon atoms per molecule such as formic acid, acetic acid, propionic acid, etc. Acetic acid is the preferred low molecular weight carboxylic acid of this invention and may be either glacial acetic acid or an aqueous solution thereof, the concen-

## 2

tration of the acetic acid in the aqueous solution varying from about 60 to 99.9 wt. percent. Substituted acetic acids having two carbon atoms per molecule such as chloro-acetic acid, glycolic acid, thioglycolic acid, glycine, etc. may also be used to modify the structure of lubricating compositions made in accordance with this invention. The amount of low molecular weight carboxylic acid employed will be within the range of about 5 to 20 wt. percent, preferably about 10 to 15 wt. percent, based on the total lubricating composition.

The mineral acids which may be employed in this invention include phosphoric acid, nitric acid, sulphuric acid, hydrochloric acid and mixtures of any combination of these acids. The concentrations of the mineral acids may vary from about 5% to 100%. The strong inorganic acids are utilized in amounts ranging from about 3 to 15 wt. percent, preferably about 5 to 10 wt. percent, based on the total lubricating composition.

The stabilizing agent of this invention is an aluminum soap of a high molecular weight carboxylic acid having from about 16 to 22 carbon atoms per molecule. Aluminum stearate is preferred, though soaps of palmitic acid, arachidic acid, behenic acid, etc. may also be employed to stabilize the lubricating grease compositions of this invention. Only stabilizing proportions of the aluminum soap of from about 2 to 10 wt. percent, preferably about 3 to 6 wt. percent, based on the total lubricating composition, need be used.

Suitable metal bases for neutralizing the blends of low molecular weight carboxylic acids and mineral acids include the alkaline earth metals: calcium, barium, magnesium and strontium; and the alkali metals: sodium, potassium and lithium. The alkaline earth metals are preferred, and calcium is especially preferred. Ordinarily, the grease-making process of this invention will utilize from about 10 to 20 wt. percent based on the total lubricating composition, of the metal hydroxide or carbonate. Mixtures of the above metals may also be employed, if desired.

The lubricating oils employed as the menstrua of the lubricating compositions of this invention may be either conventional grease-making mineral oils or synthetic lubricating oils. In general, the mineral and synthetic lubricating oils should have a viscosity within the range of about 50 to 2000 S. U. S. at 100° F. and about 30 to 200 S. U. S. at 210° F., an ASTM pour point of about +20 to -75° F., a flash point of about 350° to 650° F., and a viscosity index of about 0 to 60, although lubricating oils having a viscosity index of 100 or higher can also be employed. When a strong acid like nitric or sulphuric is used in high concentrations according to the present invention, the preferred menstrum is a mineral lubricating oil.

The synthetic lubricating oils include esters of mono-basic acids (e. g. an ester of C<sub>8</sub> alcohol with C<sub>8</sub> Oxo acid, an ester of C<sub>12</sub> Oxo alcohol with octanoic acid, etc.), esters of dibasic acids (e. g. di-2-ethyl hexyl sebacate, dinonyl adipate, etc.), esters of glycols (e. g. C<sub>12</sub> Oxo acid diester of tetraethylene glycol, etc.), complex esters (e. g. the complex ester formed by reacting one mole of tetraethylene glycol with two moles of sebacic acid and two moles of 2-ethyl-hexanol, a complex ester formed by reacting one mole of azelaic acid, one mole of tetraethylene glycol, one mole of C<sub>8</sub> Oxo alcohol and one mole of C<sub>8</sub> Oxo acid), esters of phosphoric acid (e. g. the ester formed by contacting three moles of the mono-methyl ether of ethylene glycol with one mole of phosphorous oxychloride, etc.), halocarbon oils (e. g. the polymer of

chlorotrifluoroethylene containing twelve recurring units of chlorotrifluoroethylene), alkyl silicates (e. g. methyl polysiloxanes, ethyl polysiloxanes, methyl-phenyl polysiloxanes, etc.), sulfite esters (e. g. ester formed by reacting one mole of sulfur oxychloride with two moles of the methyl ether of ethylene glycol, etc.), carbonates (e. g. the carbonate formed by reacting  $C_8$  Oxo alcohol with ethyl carbonate to form a half ester and reacting this half ester with tetraethylene glycol), mercaptals (e. g. the mercaptal formed by reacting 2-ethyl hexyl mercaptan with formaldehyde), formals (e. g. the formal formed by reacting  $C_{13}$  Oxo alcohol with formaldehyde), polyglycol type synthetic oils (e. g. the compounds formed by condensing butyl alcohol with fourteen units of propylene oxide, etc.), or mixtures of the above in any proportions.

The lubricating compositions of the invention will contain about 50 to 90 wt. percent, preferably about 60 to 80 wt. percent, of the mineral and/or synthetic lubricating oil and about 10 to 50 wt. percent, preferably about 20 to 40 wt. percent of the reaction products of blends of the above acids with the metal base plus the aluminum soap.

In general, the lubricating grease compositions of this invention may be prepared by coneutralization of a blend of the low molecular weight carboxylic acid and the mineral acid in a lubricating oil containing a minor amount of the aluminum soap. No external heating is required during the coneutralization step, since the reactions taking place are exothermic. In practice, the temperature following the addition of the blend of acids will rise to about 190° to 216° F., and a solid grease forms almost immediately.

The preferred method for preparing the lubricating compositions of the invention involves dispersing the aluminum soap in the lubricating oil at a temperature of from about 270° to 350° F. with stirring. The resulting dispersion is cooled to room temperature, preferably by pan cooling. The cold aluminum soap-lubricating oil dispersion is then charged to a grease kettle equipped with means for efficient stirring. The metal hydroxide is added with stirring to obtain a smooth uniform slurry. The low molecular weight carboxylic acid blended with the mineral acid is then added to the grease kettle with stirring. A solid grease forms almost immediately without the application of external heat. Stirring is continued until the temperature subsides from about 180° to 210° F. to about 100° to 140° F. The resulting grease composition may be finished by passage through a Morehouse mill or Gaulin homogenizer at high rates of shear.

Only a portion of the total lubricating oil required to prepare the compositions of this invention need be initially employed to disperse the aluminum soap and the blend of acids. The remainder of the lubricating oil can be conveniently added subsequent to the addition of the blend of low molecular weight carboxylic acids and mineral acids.

When a portion of the lubricating oil is a saponifiable synthetic oil, it is preferred to initially disperse the reactants in a mineral oil or the non-saponifiable synthetic oil portion of the lubricating oil, and to then add the saponifiable synthetic oil to the grease batch after the latter has been cooled.

Conventional lubricating grease additives may also be employed in the lubricating compositions of the present invention. These additives, for example, include: oxidation inhibitors, such as phenyl alpha naphthylamine, corrosion inhibitors such as sorbitan monooleate, tackiness agents such as polyisobutene or high molecular weight polymerized acrylic esters, load-carrying compounds such as sulfurized and/or phosphorous and/or chlorine containing oil-soluble materials, and the like.

The invention will be more fully understood by reference to the following specific examples illustrating various modifications of the invention.

## EXAMPLE I

A lubricating grease composition according to this invention was prepared from the following constituents:

|    |                                          | Percent weight |
|----|------------------------------------------|----------------|
| 5  | Formulation:                             |                |
|    | Glacial acetic acid                      | 14.0           |
|    | Phosphoric acid (85% conc.)              | 6.0            |
|    | Hydrated lime                            | 15.0           |
|    | Aluminum stearate                        | 3.2            |
| 10 | Phenyl alpha naphthylamine               | 0.5            |
|    | Mineral lubricating oil 55 SUS @ 210° F. | 61.3           |

## Preparation

The aluminum stearate was dispersed in all of the mineral lubricating oil by heating to a temperature of about 300° F. with stirring. The resulting dispersion was cooled to room temperature in pans. Just prior to drawing into the pans, the phenyl alpha naphthylamine was added to the dispersion. The cooled dispersion was then charged to a grease kettle, and the lime added with mixing to obtain a smooth uniform slurry. A blend of the acetic acid and the phosphoric acid was then charged to the grease kettle. Without heating the resulting grease batch, the temperature rose to about 190° F. Stirring was continued until the temperature subsided, and the grease was finished by being passed through a Gaulin homogenizer.

## Properties

|                                    |                                                                                     |
|------------------------------------|-------------------------------------------------------------------------------------|
| Appearance                         | Excellent, smooth uniform grease.                                                   |
| Dropping point, ° F.               | 400+.                                                                               |
| 30 Penetration 77° F. mm./10:      |                                                                                     |
| Unworked                           | 190.                                                                                |
| Worked 60 strokes                  | 210.                                                                                |
| Worked 70,000 strokes              | 235.                                                                                |
| Water solubility                   | Nil.                                                                                |
| Water renellency (175° F.)         | Excellent.                                                                          |
| Phase changes up to 400° F.        | After removal of water, grease becomes somewhat softer but does not lose structure. |
| 35 Norma Hoffman oxidation test    | 335.                                                                                |
| (hrs. to 5 p. s. i. drop)          |                                                                                     |
| Lubrication life (hours) (250° F.) | 1000+. <sup>1</sup>                                                                 |
| 10,000 R. P. M.)                   |                                                                                     |

<sup>1</sup> Not a lubrication failure, test discontinued; the bearings and greases were still in good condition.

It will be noted from the above data that lubricating greases of this invention are readily suitable for lubricating services at elevated temperatures and under various operating conditions. It is also apparent that greases prepared in accordance with this invention are also sufficiently economical to compete with conventional cup greases.

## EXAMPLE II

|    |                                          | Percent weight |
|----|------------------------------------------|----------------|
| 50 | Formulation:                             |                |
|    | Glacial acetic acid                      | 14.0           |
|    | Nitric acid (70% conc.)                  | 8.6            |
|    | Hydrated lime                            | 15.1           |
|    | Aluminum stearate                        | 3.1            |
| 55 | Phenyl alpha naphthylamine               | 0.6            |
|    | Mineral lubricating oil 55 SUS @ 210° F. | 58.6           |

## Preparation

Similar to that described in Example I, except that nitric acid was employed in place of the phosphoric acid.

|                                    |                                                                                                               | Properties |
|------------------------------------|---------------------------------------------------------------------------------------------------------------|------------|
| Appearance                         | Excellent, smooth uniform red product.                                                                        |            |
| Penetrations, 77° F., mm./10:      |                                                                                                               |            |
| Unworked                           | 200.                                                                                                          |            |
| Worked 60 strokes                  | 230.                                                                                                          |            |
| Worked 70,000 strokes              | 260.                                                                                                          |            |
| Dropping point, ° F.               | 400+.                                                                                                         |            |
| Water solubility (boiling water)   | No turbidity after 10 minutes boiling.                                                                        |            |
| Phase changes up to 400° F.        | Grease softens after removal of water but does not lose structure. Semi-fluid on cooling to room temperature. |            |
| 70 Norma Hoffman oxidation test    | 250.                                                                                                          |            |
| (hrs. to 5 p. s. i. drop)          |                                                                                                               |            |
| Lubrication life (hours) (250° F.) | 850.                                                                                                          |            |
| 10,000 R. P. M.)                   |                                                                                                               |            |

The above data shows that mineral acids other than phosphoric acid can be effectively employed to prepare lubricating grease compositions in combination with low

molecular weight carboxylic acids. It will be further noted that when nitric acid is employed, the resulting grease composition had a red color indicating that this strong inorganic acid may have reacted in some manner with the lubricating oil base.

It will be further understood that the present invention is not necessarily limited to the specific materials and conditions of the foregoing examples. These materials and conditions may be varied within the limits indicated in the general portions of the specification.

What is claimed is:

1. A lubricating composition comprising a major amount of a lubricating oil, and an alkaline earth metal neutralized blend of 5 to 20 wt. percent low molecular weight carboxylic acid having from about 1 to 3 carbon atoms per molecule and 3 to 15 wt. percent mineral acid, and 3 to 6 wt. percent aluminum soap, all of said weight percentages being based on the total weight of the lubricating composition.

2. The lubricating composition of claim 1 wherein said lubricating oil is a mineral lubricating oil.

3. The lubricating composition of claim 1 wherein said alkaline earth metal is calcium.

4. The lubricating composition of claim 1 wherein said mineral acid is selected from the group consisting of phosphoric acid, nitric acid, hydrochloric acid, sulfuric acid, and mixtures thereof.

5. The lubricating composition of claim 1 wherein said aluminum soap is an aluminum soap of a high molecular weight carboxylic acid having from about 16 to 22 carbon atoms per molecule.

6. The method of preparing a lubricating grease composition which consists essentially of dispersing an aluminum soap of a high molecular weight carboxylic acid having from about 16 to 22 carbon atoms per molecule in a lubricating oil by heating, cooling said dispersion to 10 ambient temperature, adding an alkaline earth metal hydroxide to said cooled dispersion, then adding a blend of a low molecular weight carboxylic acid having from about 1 to 3 carbon atoms per molecule and a mineral acid to the resulting mixture to obtain said lubricating 15 grease composition.

7. The method of claim 6 wherein said aluminum soap is aluminum stearate.

8. The method of claim 6 wherein said low molecular weight carboxylic acid is acetic acid.

9. The method of claim 6 wherein said mineral acid is nitric acid.

References Cited in the file of this patent

UNITED STATES PATENTS

25 2,417,429 McLennan Mar. 18, 1947